

Jan. 14, 1930.

C. P. BEATH ET AL

1,743,309

ALLOY OF STEEL AND METHOD OF TREATING THE ALLOY

Filed Nov. 19, 1927



Inventors  
Charles P. Beath  
Bethel J. Babbitt  
by H. F. Luttmann Atty.

## UNITED STATES PATENT OFFICE

CHARLES PHILIP BEATH, OF LA GRANGE, AND BETHEL JAY BABBITT, OF RIVERSIDE, ILLINOIS, ASSIGNEES TO WESTERN ELECTRIC COMPANY, INCORPORATED, OF NEW YORK, N. Y., A CORPORATION OF NEW YORK

## ALLOY OF STEEL AND METHOD OF TREATING THE ALLOY

Application filed November 19, 1927. Serial No. 234,336.

This invention relates to an alloy of steel and a method of treating the alloy, and more particularly to a magnet steel alloy and a method of heat treating the alloy.

5 The objects of the invention are to provide a magnet steel having a high remanence and coercive force and an improved method of treating the magnet steel.

In accordance with the general features 10 of the invention, the magnet steel consists chiefly of the ferrous metals comprising iron, cobalt, and nickel which may be magnetically hardened to obtain a high coercive force and magnetic remanence by heating the steel for 15 a prolonged period and then quenching the steel at a temperature not in excess of 1550° F.

Ores containing cobalt in many cases also contain considerable quantities of nickel, iron and carbon. It has been found that a 20 high quality of magnet steel having the required remanence and coercive force can be produced without fully refining such ores by removing certain constituents and adding others and subjecting the resulting alloy to 25 an appropriate heat treatment.

For an illustration of the characteristics 30 of the magnet steel of this invention reference may be had to the accompanying drawing in which the single figure graphically represents the improvement of the magnetic properties of the steel upon a prolonged heat treatment. The abscissas in the figure represent hardening temperatures and the ordinates for the maximum and residual induction indicated at the left side of the figure represent magnetic induction in maxwells per square centimeter, while the ordinates for coercive force indicated at the right side of the figure represent the magnetic coercive 40 force in giberts per centimeter.

Curve 2 represents the maximum induction of a specimen of magnet steel of this invention showing the specimen to have a maximum induction when hardened at a temperature in the vicinity of 1550° F. Curve 3 represents the maximum induction of a similar specimen after retaining it at the hardening temperature for two or three hours before quenching. It will be noted that the prolonged heating of the specimen reduces the

hardening temperature and increases the magnetic induction of the steel. A similar but even more pronounced effect of the prolonged heating is had upon the magnetic remanence of the steel as may be seen from 55 curves 4 and 5 representing the residual magnetic induction of a specimen not heat treated and a heat treated specimen respectively. The curve of the heat treated specimen shows that its residual magnetism is from 800 to 1000 maxwells per square centimeter greater than the residual magnetism of the specimen which has not been heat treated, and since residual magnetism determines the strength 60 of a permanent magnet this effect is of considerable importance.

The curves 6 and 7 show the effect of the heat treatment upon the coercive force of the steel. In contrast to the maximum and residual induction the hardening temperature is slightly greater for a given coercive force and the coercive force is slightly decreased in the heat treated specimen until the curves reach the temperature of approximately 1500° F. where they meet. If, therefore, the 70 steel is hardened at a temperature in the vicinity of 1500° F. the coercive forces will be the same in a heat treated specimen and one that has not been heat treated while in the former the residual and maximum induction 75 will be greatly increased.

The preferred form of the magnet steel alloy consists of cobalt 20%, tungsten 9%, manganese 2.5%, carbon .8%, nickel 7% and 80 60.7% iron. These proportions may be varied to some extent, and the alloy will still retain its essential characteristics. Thus the cobalt content may be varied from 5 to 50%, the tungsten content from 1 to 12%, the manganese content from 0 to 7%, the carbon content from .3 to 5%, and the nickel content from 6 to 18%. The alloy may also contain chromium from 0 to 12%.

The nickel content of this alloy has an important effect in its heat treatment. Many steels depreciate considerably when exposed to high temperatures for an extended time. As pointed out above the magnetic characteristics of the steel of this invention improve 95 100

when the steel is retained at a high temperature for several hours.

In the heat treatment of the magnet steel of this invention the steel is formed into the shape which the finished magnet is to possess and its temperature is raised above the  $A^2$  transformation point. The metal is then retained at a temperature of approximately  $1500^{\circ}$  to  $1550^{\circ}$  F. for two to three hours when it is quenched in air, water, oil, or other suitable quenching medium. The quenching of the steel at this temperature imparts to it the desired magnetic characteristics of possessing a high coercive force and magnetic remanence.

It will be understood that the embodiments of the invention herein described and illustrated are merely representative forms of the invention which is capable of many other modifications without departing from the spirit of the invention.

What is claimed is:

1. A magnet steel alloy comprising cobalt 5-50%, tungsten 1-12%, manganese 0-7%, carbon .3-5%, nickel 5-18%, chromium 0-12%, and iron.

2. A magnet steel alloy comprising cobalt 20%, tungsten 9%, manganese 2.5%, carbon .8%, nickel 7%, and iron 60.7%.

3. A method of improving the magnetic properties of a cobalt-nickel steel, which consists of heating a steel containing 5 to 50% cobalt and 5 to 18% nickel to a temperature above the  $A^2$  transformation point, allowing the steel to cool to a temperature of approximately  $1500^{\circ}$  F., and quenching the steel.

4. A method of improving the magnetic properties of a cobalt-nickel steel, which consists of heating a steel containing 5 to 50% cobalt and 5 to 18% nickel to a temperature above the  $A^2$  transformation point, retaining the temperature at from  $1500$  to  $1550^{\circ}$  F. for several hours, and quenching the steel.

5. A method of producing a high coercive force and a high magnetic remanence in a cobalt-nickel steel, which consists of heating a steel containing 5 to 50% cobalt and 5 to 18% nickel to a temperature above the  $A^2$  transformation point, retaining the temperature at approximately  $1500^{\circ}$  F. for two to three hours, and quenching the steel.

6. A method of producing a high coercive force and high magnetic remanence in a cobalt-nickel steel, which consists of heating a steel containing 5 to 50% cobalt, 1 to 12% tungsten, 0 to 7% manganese, .3 to 5% carbon, 5 to 18% nickel, 0 to 12% chromium and the remainder principally iron, to a temperature above the  $A^2$  transformation point, allowing the steel to cool to a temperature of approximately  $1500^{\circ}$  F., and quenching the steel.

7. A method of producing a high coercive force and high magnetic remanence in a co-

balt-nickel steel, which consists of heating a steel containing approximately 20% cobalt, 9% tungsten, 2.5% manganese, .8% carbon, 7% nickel and 60.7% iron to a temperature above the  $A^2$  transformation point, retaining the temperature at approximately  $1500^{\circ}$  F. for two to three hours, and quenching the steel.

In witness whereof, we hereunto subscribe our names this 7th day of November A. D., 1927.

CHARLES PHILIP BEATH.  
BETHEL JAY BABBITT.

80

85

90

95

100

105

110

115

120

125

130

70

75

80

85

90

95

100

105

110

115

120

125

130